# EUROPEAN PATENT SPECIFICATION

(11) **EP 0 050 766 B1**
(45) Date of publication and mention of the grant of the patent: **31.07.1985**
(21) Application number: 81108092.8
(22) Date of filing: 09.10.1981
(51) Int. Cl.: D21F 1/00

(54) **Dryer fabric and method of making it**
Trocknergewebe sowie Verfahren zu dessen Herstellung
Tissu de séchage et son procédé de fabrication

(30) Priority: 16.10.1980 US 197551
(43) Date of publication of application: 05.05.1982
(73) Proprietor: Huyck Corporation, Wake Forest North Carolina 27587 (US)
(72) Inventor: Mullaney, Peter, Raleigh North Carolina (US)
(74) Representative: Hoeger, Stellrecht & Partner

## Description

### Technical field

The invention is directed to a fluid-permeable, woven dryer fabric for use in a papermaking machine, being woven of machine direction yarns and cross machine direction yarns in a multilayer weave with said machine direction yarns being evenly spaced along the width of the dryer fabric and with additional yarns being located in said dryer fabric at selected positions across the width of the dryer fabric to produce longitudinally extending zones in said dryer fabric across the width thereof having different fluid permeabilities and to a method for making it.

### Background art

The usual papermaking machine has three primary sections; a forming section, a press section and a drying section. In the forming section, wet pulp is deposited on the forming surface of a forming fabric which is of the nature of a fluid-permeable endless belt. Vacuum is applied to the underside of the forming fabric to withdraw moisture from the pulp, causing the pulp to form a sheet on the forming fabric. From the forming section, the sheet is transferred to the press section and is conveyed by a press fabric through a series of press rolls to further remove water from the web. From the press section, the web is then transferred to the dryer section where it is passed about a series of heated dryer cylinders. One or more dryer fabrics are employed to press the moist web uniformly and successively against the dryer cylinders to dry the web. As used herein and in the claims, the term "papermaking machine" is to be considered in a broad or generic sense, the machine producing a paper or paper-like material such as pulp, board, asbestos sheet or other similar structures.

In the dryer section, the dryer cylinders are internally heated by steam or the like. The cylinders usually have imperforate surfaces for contacting the paper web. Other rolls, such as packet rolls may have surfaces which are perforated or slotted to permit the passage of heated air therethrough to increase the drying action on the web.

Several problems are encountered in the dryer section. First of all, it has been found that the surface temperature of the dryer cylinders may vary axially across the machine direction by as much as 22°C. This produces the distinct possibility that some portions of the web will be subjected to greater drying action than other portions of the web, resulting in a non-uniform moisture profile across the web.

A second problem results from the fact that moisture from the paper web tends to collect in enclosed areas or "pockets" in the dryer section. Usually more moisture accumulates in the central portions of the pockets than in those portions of the pockets lying nearer the lateral edges of the dryer section, the portions nearer the lateral edges of the drying section being more readily ventilated by the surrounding atmosphere.

Thus, by virtue of the variance in temperature across the cross machine direction or the dryer cylinders and moisture accumulated in pockets in the dryer section, the web generally will have a higher moisture content near its center, than at its edges. This is undesirable from the standpoint of quality control of the end product. Prior art workers have taken numerous steps to alleviate this problem. First of all, dryer fabrics have been devised which are fluid-permeable, such dryer fabrics having an open weave. An exemplary open weave dryer fabric is taught in US-A-2,180,054. Dryer fabrics in the form of nonwoven structures such as needled felts and perforated plastic belts have also been used. To further alleviate the problem, various types of air jet apparatus or exhaust means have been provided to eliminate moisture build-up in the dryer pockets. Such devices are generally extremely complex and difficult to maintain, particularly in new dryer sections capable of handling webs having a width of the order of 10 m.

Yet another approach to the provision of a more uniform moisture profile across the web is taught in US-A-3,867,766. According to the teachings of this reference, a fluid permeable dryer fabric is provided, the permeability of which varies at selected locations across its width. This is accomplished in several ways. In a first embodiment, the machine direction yarns in the edge regions of the dryer fabric are more closely spaced with respect to one another than in the center region of the dryer fabric. It is to be noted that the phrase "machine direction" used herein and in the claims refers to the direction of travel of the dryer fabric when mounted in the dryer section of the papermaking machine. The phrase "cross machine direction" refers to that direction transverse the dryer fabric and perpendicular to the direction of travel of the dryer fabric in the dryer section of the papermaking machine.

In another embodiment, US-A-3,867,766 teaches selectively varying the diameter of the machine direction yarns so that those yarns which lie in the area desired to be of reduced permeability have a diameter greater than those machine-direction yarns located in the more permeable sections of the dryer fabric. In a third embodiment, this reference teaches the utilization of machine direction yarns having a higher bulk construction near the lateral edges of the dryer fabric. These yarns will tend to flatten and close off the effective open area between adjacent yarns, thus reducing the permeability of the dryer fabric near its edges. In a final embodiment, the dryer fabric is selectively treated with greater amounts of resin or the like at its edges, than in its center, to reduce permeability at the edges thereof.

The various approaches taught in the above mentioned US-A-;3,867,766, while effective, have certain drawbacks. For example, when the frequency of machine direction yarns is increased at the edges of the dryer fabric, the edges tend to resist stretch to a greater extent and operate at a higher tension than the center of the dryer fabric. Furthermore, as the machine direction yarns elongate and loose crimp, the cross machine direction yarns must accept crimp. However, the cross machine direction yarns are more difficult to bend as their ability to accept crimp is a function of the distance between the machine direction yarns. As a result, it has been found that dryer fabrics of the type taught in US-A-3,867,766 demonstrate differences in machine direction physical characteristics across the width of the dryer fabric. These differences in machine direction physical characteristics between sections of differing end counts present problems in achieving uniform flatness across the width of the dryer fabric and, similarly, can give rise to difficulties in running flat and wrinkle free in the dryer section of the papermaking machine. Furthermore, it is generally accepted that higher operating tension in a dryer fabric gives rise to increased drying of the web. Therefore, dryer fabrics in which the edge portions have a higher frequency of machine direction yarns, to reduce the permeability and thereby the drying rate of the edge portions of the fabric, suffer some counteracting effects of increased drying of the web at the fabric edges due to their edges operating at a higher tension.

The use of one or more resin coatings on the dryer fabric to vary its permeability across its width has not proven very effective due to the difficulty in maintaining the resin coating throughout the life of the fabric. This is even more difficult to achieve in dryer fabrics made of monofilament yarns, due to the resistance of monofilament yarns to the acceptance of resin coatings.

Further, FR-A-2024 388 describes a woven dryer fabric of the type indicated above, wherein said additional yarns are laid in machine direction for the purpose of different permeability across the width of the dryer fabric. It has been found that the known dryer fabric is not entirely satisfactory in all cases, especially regarding the method of producing the same.

FR-A-2 407 291 shows additional cross direction yarns (weft-yarns) in a dryer fabric but only to influence the permeability in width as a whole which in some cases also is not satisfactory.

The present invention is based upon the discovery that if, in a woven dryer fabric, additional cross machine direction yarns, which may be of various thicknesses or bulk, are located in the fabric at selected positions across the fabric, the permeability of the dryer fabric can be varied by design, in different sections across its width. The additional cross machine direction yarns have little or no effect on the machine direction load bearing properties of the dryer fabric. Thus, there will be no substantial differences in machine direction physical characteristics between the sections of the dryer fabric having different permeabilities. Furthermore, the present invention can be practiced in the manufacture of dryer fabrics made substantially from monofilament yarns. The dryer fabrics of the present invention can also be pinseamed.

A well known problem encountered in the dryer section of a papermaking machine is frequently referred to as "edge flutter" in the web. This problem is more severe at the web edges and tends to limit the speed at which the dryer section of the papermaking machine can be run. The dryer fabrics of the present invention provide much better control of edge flutter in the web and therefore permit the dryer section to be run at higher speeds.

Another well known problem in the art is a malformation in the web edges known as "grainy edges" or "cockled edges" due to greater drying of the web at the edges and flutter. The dryer fabrics of the present invention tend to reduce or eliminate such malformations in the web edges.

Woven dryer fabrics are used in the dryer section of the papermaking machine in the form of endless belts. To this end, the dryer fabrics may be woven directly in the form of endless belts by endless weaving techniques well known in the art. In such an instance, the weft or filling yarns extend in the machine direction and the warp yarns extend in the cross machine direction. Alternatively, the dryer fabrics can be flat woven with their ends joined by well known means to form continuous belts. When the dryer fabrics are flat woven, the warp yarns extend in the machine direction and the weft or filling yarns extend in the cross machine direction. While the dryer fabrics of the present invention can be woven by either technique, for purposes of an exemplary showing the dryer fabrics will be described herein in terms of flat woven fabrics.

Proceeding on the basis of the prior art, especially according to FR-A-2 024 388, it is the object of this invention to provide an improved dryer fabric, wherein the additional yarns being provided for the purpose of different permeability across the width of the dryer fabric have little or no effect on the machine direction load bearing properties of the dryer fabric. This object is accomplished with a dryer fabric of the type indicated above which according to the invention is characterized in that the additional yarns are stuffer picks laid in cross machine direction and being of a length shorter than the width of the dryer fabric..

In a first embodiment, the dryer fabric is woven utilizing any appropriate multi-layer weave and stuffer picks are introduced into the weave at edge sections of the dryer fabric. The stuffer picks extend from the dryer fabric edges inwardly in a cross machine direction for a predetermined distance toward the center of the fabric. This provides a dryer fabric having a central section of high permeability and edge sections of lesser permeability.

In a second embodiment, stuffer picks are introduced in the edge sections of the dryer fabric, as in the first embodiment. Additional stuffer picks of lesser diameter or less bulk are introduced into the center section of the dryer fabric, extending in the cross machine direction between opposed edge section stuffer picks. The resulting dryer fabric of this second embodiment differs from the first embodiment in that the center section of the dryer fabric has a somewhat reduced permeability, although the center section is still of greater permeability than the edge sections of the dryer fabric.

In a third embodiment, stuffer picks are again introduced at the edge portions of the dryer fabric. In this instance, however, alternate opposed pairs of stuffer picks at the edge sections are longer than the remaining edge stuffer picks. Again, additional stuffer picks of lesser diameter or less bulk are introduced into the dryer fabric extending between opposed edge stuffer picks. This provides a dryer fabric having edge sections containing the larger diameter stuffer picks, a center section containing the stuffer picks of less diameter or bulk and two intermediate sections containing alternate large diameter stuffer picks and stuffer picks of lesser diameter or bulk. As a consequence, the dryer fabric has five sections across its width of differing permeabilities. The centermost section has the greatest permeability. To either side of the center sections are sections of intermediate permeability and at the edges are sections of the least permeability.

A fourth embodiment of the present invention is identical to the third embodiment with the exception that the stuffer picks of lesser diameter or bulk are omitted. This again yields a five section dryer fabric with the centermost section having maximum permeability.

In all of the embodiments of the present invention the width of the sections of the dryer fabric of differing permeabilities does not constitute a limitation. The various sections can be made of any appropriate width depending upon the ultimate conditions of use of the dryer fabric, the material being dried, the axial temperature variance of the dryer rolls, and the like. Similarly, the nature of the yarns from which the dryer fabric is woven does not constitute a limitation. Spun yarns, monofilament yarns, multifilament yarns and combinations thereof can be used.

### Brief description of the drawings

Figure 1 is a semi-diagrammatic representation of an exemplary dryer section of a papermaking machine.
Figure 2 is a fragmentary, semi-diagrammatic plan view of a first embodiment of dryer fabric of the present invention.
Figure 3 is a fragmentary, semi-diagrammatic cross sectional view taken along section line 3-3 of Figure 2.
Figure 4 is a fragmentary, semi-diagrammatic cross-sectional view taken along section line 4-4 of Figure 2.
Figure 5 is a fragmentary, semi-diagrammatic plan view of a second embodiment of dryer fabric of the present invention.
Figure 6 is a fragmentary, semi-diagrammatic cross sectional view taken along section line 6-6 of Figure 5.
Figure 7 is a fragmentary semi-diagrammatic plan view of a third embodiment of the dryer fabric of the present invention.
Figure 8 is a fragmentary, semi-diagrammatic cross sectional view taken along section line 8-8 of Figure 7.
Figure 9 is a fragmentary, semi-diagrammatic plan view of a fourth embodiment of the dryer fabric of the present invention.
Figure 10 is a fragmentary, semi-diagrammatic cross-sectional view taken along section line 10-10 of Figure 9.

### Best mode of carrying out the invention

Reference is first made to Figure 1 wherein an exemplary dryer section of a papermaking machine is shown. The dryer section is made up of an upper array of drying cylinders 1, 2 and 3 a lower array of drying cylinders 4 and 5. The drying cylinders 1 through 5 are heated by an appropriate means such as steam or the like. As indicated above, other rolls, such as rolls 9 and 11, may have imperforate surfaces, or perforated surfaces to permit the passage therethrough and through the web to be dried of heated air.

In Figure 1, a web to be dried is shown at 6. The web has an upper surface 6a and a lower surface 6b. The web is guided to and from the dryer section by guide rolls 7. As indicated above, the web 6 may be of any material normally made in a papermaking or papermaking-like machine including paper, pulp, board, asbestos sheet or the like. It will be noted from Figure 1 that the web travels through the dryer section in a senuous path, contacting each of the upper and lower dryer cylinders in order. It will further be noted that the upper surface 6a of web 6 is contacted by the cylinders 4 and 5 of the lower array, and the lower surface 6b of the web is contacted by cylinders 1, 2 and 3 of the upper array.

The dryer section of Figure 1 is of the type utilizing two dryer fabrics. A first dryer fabric 8 is shown passing about portions of the upper array of cylinders 1, 2 and 3. The dryer fabric is appropriately guided and tensioned by additional pocket rolls 9. The purpose of the upper dryer fabric 8 is to bear upon web 6 as it passes about cylinders 1, 2 and 3, bringing the underside 6b of the web into intimate contact with the cylinders 1, 2 and 3.

A lower dryer fabric 10 passes about portions of the cylinders 4 and 5 of the lower array and is appropriately tension and guided by pockets rolls 11. Again, the purpose of lower dryer fabric 10 is to press the web 6 against dryer cylinders 4 and 5, bringing the upper surface 6a of the web into intimate contact with dryer cylinders 4 and 5. It will be understood that the dryer fabrics 8 and 10 are substantially identical, except for length, and the teachings of the present invention are applicable to either the upper or the lower dryer fabrics.

A first embodiment of the present invention is illustrated in Figures 2, 3 and 4, wherein like parts have been given like index numerals. Reference is first made to Figures 2 and 3. The dryer fabrics of the present invention are woven of yarns and the yarns may be spun yarns, monofilament yarns, multifilament yarns or combinations thereof. As indicated above, for purposes of an exemplary showing only, the dryer fabrics of the present invention will be described as flat woven.

It is a requirement of the present invention that the dryer fabrics be woven, utilizing a multi-layer weave. To this end, the embodiment of Figures 2, 3 and 4, generally indicated at 12, is shown in diagrammatic fashion as being made of a simple duplex weave. The warp or machine direction yarns are shown at 13. The weft or filling yarns (cross machine direction yarns) are arranged in two layers. The upper fitting yarns are indicated at 14 and the lower filling yarns are shown at 15. Since the yarns 14 and 15 are arranged in vertical pairs, only yarns 14 are visible in Figure 2. Both layers of filling yarns are shown in Figures 3 and 4.

It will be evident from the semi-diagrammatic representation of the simple duplex weave in Figure 3 that a series of diamond-shaped openings occur between the vertical pairs of filling yarns 14 and 15. These diamond-shaped openings are shown at 16.

In the embodiment of Figures 2 through 4, stuffer picks are inserted in the diamond-shaped openings 16. The stuffer picks are illustrated at 17 in Figure 4. As is most clearly shown in Figures 2, the stuffer picks 17 extend from the longitudinal edges of the dryer fabric 12 for a predetermined distance toward the center of the dryer fabric. It will be immediately evident from Figure 2 that the dryer fabric 12 has three sections or zones. Edge sections 18 and 19 contain the stuffer picks 17. A central section or zone 20 is devoid of stuffer picks. As a result of the presence of stuffer picks 17 in sections 18 and 19, these sections will have a fluid permeability less than central section 20.

It will be understood by one skilled in the art that the width of sections 18, 19 and 20 does not constitute a limitation on the present invention. During the weaving process, sections 18, 19 and 20 may be tailored to have any desired width so that the dryer fabric 12 may have a cross machine direction permeability profile tailored to its particular end use. The width of sections 18, 19 and 20 will depend upon a number of factors such as the nature of the material from which the web 6 is made, the desired moisture profile for the dried web, the temperature variance along the axial length of dryer cylinders 1 through 5 in the cross machine direction, the yarns from which the dryer fabric is made, the width of the dryer fabric and the web 6, etc.

Figures 5 and 6 illustrate a second embodiment of the present invention. In this embodiment, the dryer fabric is generally indicated at 12a. Dryer fabric 12a is substantially identical to dryer fabric 12 of Figures 2 through 4 and like parts have been given like index numerals. The dryer fabric 12a has warp or machine direction yarns 13, weft or filling yarns 14 and 15 in the cross machine direction and stuffer picks 17 extending inwardly from both longitudinal sides of the dryer fabric. As a result, the dryer fabric 12a is again divided into two edge zones 18a, and 19a and a central zone 20a. The only difference between the dryer fabric 12a of Figures 5 and 6 and the dryer fabric 12 of Figures 2 through 4 lies in the fact that additional stuffer picks are located in the central section or zone 20a. Each of the additional stuffer picks 21 extends the full width of the central section 20a and are in general alignment with the opposed edge stuffer picks 17 which occupy the same diamond-shaped opening 16.

Figure 4 may be considered to be a longitudinal cross sectional view through either of the sections or zones 18a or 19a of Figure 5. Figure 6 is a longitudinal cross sectional view through the central zone 20a of Figure 5. It will be immediately apparent that the stuffer picks 21 are so selected as to have a smaller size or less bulk than stuffer picks 17. As a result, the dryer fabric 12a will differ from dryer fabric 12 in that the central zone or section 20a will have a somewhat lesser permeability than center section 20 of Figure 2, while still having a greater permeability than edge sections 18a and 19a. Again, the width of sections 18a, 19a and 20a can be varied, as described with respect to the embodiment of Figures 2 through 4.

A third embodiment of the present invention, generally indicated at 12b, is illustrated in Figures 7 and 8. For purposes of an exemplary illustration, the dryer fabric 12b is shown as being woven of a simple duplex weave. Warp or machine direction yarns are again shown at 13 and weft or filling yarns, extending in the cross machine direction, are again illustrated at 14.

As in the previous embodiments, stuffer picks are provided at the edge portions of the dryer fabric 12b. Stuffer picks similar to those of the previous embodiments are shown at 17. Fabric 12b differs from the previous embodiments in that alternate edge stuffer picks are longer, extending inwardly from the edge of the dryer fabric toward the center a greater distance. These stuffer picks are illustrated at 17a.

Dryer fabric 12b is also provided with stuffer picks of lesser diameter or bulk extending between the edge stuffer picks. Those intermediate stuffer picks extending between edge stuffer picks 17 are identical to those illustrated in Figure 5 and are again given index numeral 21. Those intermediate stuffer picks extending between elongated stuffer picks 17a are, of course, shorter and are indicated by index numeral 21a.

As a result of this construction, it will be evident from Figure 7 that the dryer fabric 12b is divided into five zones or sections across its width (i.e. in the cross machine direction). First of all, there are the edgemost sections 22 and 23. These sections are equivalent to edge sections 18 and 19 of Figure 2 and 18a and 19a of Figure 5. Therefore, the cross sectional view, Figure 4, can be considered to be illustrative of the longitudinal cross section of sections 22 and 23 of Figure 7, differing only in that alternate ones of the stuffer picks of Figure 4 would bear the index numeral 17a. These edgemost sections or zones would have the least permeability.

The centermost section 24 of dryer fabric 12b is substantially identical to the center section 20a of Figure 5, except that it is considerably narrower. The cross sectional view, Figure 6, can be considered to be illustrative of the cross section of center section 24 of Figure 7, with the exception that alternate ones of the stuffer picks of Figure 6 would be designated 21a. This is the section of dryer fabric 12b having the greatest permeability.

Finally, dryer fabric 12b has two intermediate zones or sections 25 and 26. In these zones, stuffer picks 17a and 21 alternate. The longitudinal cross section of sction 25 is shown in Figure 8. It will be understood that Figure 8 is also illustrative of the longitudinal cross section of section 26. Thus, in these sections 25 and 26 there are alternate large diameter stuffer picks and stuffer picks of lesser diameter or less bulk, yielding a permeability between that of section 24 on the one hand and sections 22 and 23 on the other. As a result, dryer fabric 12b has a high permeability center section 24, medium permeability intermediate sections 25 and 26 and lesser permeability edge sections 22 and 23.

Figures 9 and 10 illustrate a fourth embodiment of the present invention wherein the dryer fabric is designated generally at 12c. Dryer fabric 12c is identical to dryer fabric 12b of Figures 7 and 8, with the sole exception that the stuffer picks 21 and 21 a of lesser diameter or less bulk have been omitted. In Figures 9 and 10, like parts have been given the same index numerals as in Figure 7 and 8.

Once again, dryer fabric 12c is a five zone or section fabric. Thus, fabric 12c has edge zones 22 and 23 identical to edge zones 22 and 23 of fabric 12b of Figure 7. Fabric 12c has a central zone 24a, the same width as zone 24 of Figure 7, but with the lesser diameter or lesser bulk stuffer picks 21 and 21a omitted. In a similar fashion, the intermediate zones 25a and 26a of dryer fabric 12c differ from the intermediate zones 25 and 26 of dryer fabric 12b only in that the lesser diameter or lesser bulk picks 21 have been omitted.

As a result of these differences, dryer fabric 12c will have the same permeability at its edges, as does dryer fabric 12b. The central zone 24a of dryer fabric 12c will have the maximum permeability, and therefore a permeability greater than the central zone 24 of dryer fabric 12b. Figure 10 is a diagrammatic cross sectional view illustrating the longitudinal section of zone 25a of dryerfabric 12c. It will be understood that Figure 10 can also be considered to be illustrative of the longitudinal section of intermediate zone 26a of Figure 9. Since the lesser diameter or lesser bulk picks 21 are omitted in sections 25a and 26a, these sections will have a lesser permeability than center section 24a, but a greater permeability than the intermediate sections 25 and 26 of dryer fabric 12b.

The four embodiments described above are exemplary only of the manner in which the teachings of the present invention can be employed to produce dryer fabrics having zones of different permeabilities across its width (i.e., in the cross machine direction). While all of the embodiments, for purposes of an exemplary showing, have been illustrated in the form of a dryer fabric made up in a simple duplex weave, it will be understood that any appropriate multi- layer weave can be used which will enable the introduction of stuffer picks. By varying the nature of the stuffer picks and their locations, a large variety of dryer fabrics of differing permeabilities across their widths can be achieved.

Since, in accordance with the teachings of the present invention, the frequency of the warp or machine direction yarns is uniform and has not been altered across the fabric width, significant differences in load bearing characteristics across the width of the dryer fabrics have not been introduced. It is recommended that the stuffer picks not be harder or stiffer and more rigid than the base picks.

In dryer fabrics of the type taught in the above mentioned US-A-3,867,766, it has been found that the load bearing properties or stretch characteristics of the edge sections and the center section can differ in a proportion as high as 1:3.5. The dryer fabrics of the present invention demonstrate much more nearly uniform load bearing properties or stretch characteristics of the various zones across their widths.

### Example I

A dryer fabric of the type illustrated in Figure 5 was made, utilizing a simple duplex weave. The warp or machine direction yarns 13 were 508 um monofilament synthetic yarns at a frequency of 20.5 yarns per cm. Both polyester and nylon yarns were used, arranged in alternate groups of four across the width of the dryer fabric.

The filling or cross machine direction yarns 14 and 15 were 508 pm monofilament polyester yarns. The outer stuffer picks 17 were 0.7 cotton count yarns spun of polyester staple fibers. The center stuffer picks 21 were 4/4 cotton count yarns spun of polyester staple fibers. The overall pick frequency was 16 per cm, including the stuffer picks.

The dryer fabric had a width of approximately 700 cm, the outer zones 18a and 19a being approximately 100 cm wide and the central zone 20a being approximately 500 cm wide. The dryer fabric was heat set in a conventional manner to heat stabilize the fabric and to achieve the final desired dimensions.

The permeabilities of the sections 18a, 19a and 20a were tested utilizing a standard Frazier air permeability tester, yielding the permeability values in cubic feet per minute per square foot of fabric at a pressure drop of 1.3 cm of water. The sections or zones 18a and 19a demonstrated a permeability of approximately 2550 dm³ per minute, while the central section 20a demonstrated a permeability of approximately 5100 dm³ per minute.

Samples from sections 18a, 19a and 20a were subjected to a standard stretch test at 0.65% elongation in the machine direction. Under these circumstances, the edge sections 18a and 19a demonstrated a force of 17.3 N per cm of width while the center sections 20a demonstrated a force of 13 N per cm of width. Thus, the difference in load bearing properties between the edge sections 18a and 19a and the center section 20a was in the proportion of 1:1.3. Thus, it can be seen that the various sections of the fabric demonstrated very nearly the same load bearing characteristics.

### Example II

A second dryer fabric of the type illustrated in Figure 9 was manufactured, utilizing a simple duplex weave. The warp or machine direction yarns 13 were 3,525 dtex continuous multifilament polyester yarns arranged at a frequency of 12.6 ends per cm. The filling or cross machine direction yarns (including the stuffer picks) were 100% fiberglass continuous multifilament yarns arranged at a frequency of 14.2 picks per cm in the edge sections 22 and 23, 11.8 picks per cm in the intermediate sections 25a and 26a and 9.45 picks per cm in the central section 24a. When subjected to the permeability tests described with respect to Example I, the edge regions 22 and 23 demonstrated a permeability of 2,832 dm³ per minute, the intermediate sections 25a and 26a demonstrated a permeability of 7788 dm³ per minute, while the central section 24a demonstrated a permeability of 11,328 dm³ per minute.

The dryer fabric of this example had an approxi-' mate of width of 711 cm, the edge sections 22 and 23 being approximately 112 cm, the intermediate sections 25a and 26a being approximately 96.5 cm and the center section 24a being approximately 295 cm. The dryer fabric was resin treated to enhance the stability of the fabric and was heat set in a conventional manner to heat stabilize the fabric and to bring it to the final required dimensions.

Samples of the five sections 22, 23, 25a, 26a and 24a were subjected to a standard stretch test, as explained in Example I above. At 1.3% elongation in the machine direction, the edge sections 22 and 23 demonstrated a force of 15.6 N per cm of width. The intermediate sections 25a and 26a demonstrated a force of 13.6 N per cm of width and center section 24a demonstrated a force of 8 pounds per inch of width. Again, it will be noted that the machine direction load bearing characteristics were very much more uniform than those of the prior art, being in the ratio of 1:1.5 between the highest and the lowest.

## Claims

1. A woven dryer fabric (12) for use in a papermaking machine, being woven of machine direction yarns (13) and cross machine direction yarns (14, 15) in a multilayer weave with said machine direction yarns (13) being evenly spaced along the width of the dryer fabric (12) and with additional yarns (17, 17a, 21, 21a) being located in said dryer fabric (12) at selected positions across the width of the dryer fabric (12) to produce longitudinally extending zones (18, 19, 20) in said dryer fabric (12) across the width thereof having different fluid permeabilities, characterized in that the additional yarns are stuffer picks (17, 17a, 21, 21a) laid in cross machine direction and being of a length shorter than the width of the dryer fabric (12).

2. The structure claimed in claim 1 wherein said machine direction yarns (13), said cross machine direction yarns (14, 15) and said stuffer picks (17, 17a, 21, 21a) are chosen from the class consisting of monofilament yarns, multifilament yarns, spun yarns and combinations thereof.

3. The structure claimed in claim 1 wherein said stuffer picks (17, 17a, 21, 21a) are of a softness and stiffness up to that of said cross machine direction yarns.

4. The structure claimed in claim 1 including first and second groups of said stuffer picks (17), the stuffer picks (17) of said first group being so located in said dryer fabric (12) as to extend from one longitudinal edge thereof toward the center thereof a predetermined distance, said second group of stuffer picks (17) being so located in said dryer fabric (12) as to extend from the other longitudinal edge thereof toward the center thereof a predetermined distance, the stuffer picks (17) of each of said groups being of the same length, said dryer fabric (12) having two edge zones (18, 19) of lesser fluid permeability and a center zone (20) therebetween of greater fluid permeability.

5. The structure claimed in claim 1, including first and second groups of said stuffer picks (17, 17a), the stuffer picks (17, 17a) of said first group being so located in said dryer fabric (12c) as to extend from one longitudinal edge thereof toward the center thereof, said stuffer picks (17, 17a) of said second group being so located in said dryer fabric (12c) as to extend from the other longitudinal edge thereof toward the center thereof, alternate ones of the stuffer picks (17a) of each of said first and second groups thereof being longer than the remaining stuffer picks (17) of said group, in each of said first and second groups said alternate longer stuffer picks (17a) being of the same length and said remaining stuffer picks (17) being of the same length, said dryer fabric (12a) having two edge zones (22, 23) of lesser fluid permeability, a center zone (24a) of higher fluid permeability and two intermediate zones (24a, 26a) of intermediate fluid permeability.

6. The structure claimed in claim 4 including a third group of said stuffer picks (21), said stuffer picks (21) of said third group being so located in said dryer fabric (12a) as to extend between said stuffer picks (17) of said first and second groups.

7. The structure claimed in claim 5 including a third group of stuffer picks (21, 21a), said stuffer picks (21,21a) of said third group being so located in said dryer fabric (12b) as to extend between said stuffer picks (17, 17a) of said first and second groups of yarns.

8. The structure claimed in claim 6 wherein said stuffer picks (21) of said third group have a diameter less than said stuffer picks (17) of said first and second groups.

9. The structure claimed in claim 6 wherein the stuffer picks (21) of said third group are of less bulk than said stuffer picks (17) of said first and second groups.

10. The structure claimed in claim 7 wherein said stuffer picks (21, 21a) of said third group have a diameter less than said stuffer picks (17, 17a) of said first and second groups.

11. The structure claimed in claim 7 wherein said stuffer picks (21, 21a) of said third group are of less bulk than said stuffer picks (17, 17a) of said first and second groups.

12. A method of making a dryer fabric (12) for use in a papermaking machine including the steps of weaving said dryer fabric (12) of machine direction yarns (13) and cross machine direction yarns (14, 15) in a multi-layer weave with said machine direction yarns (13) being evenly spaced along the width of said dryer fabric (12, and introducing additional yarns (17, 17a, 21, 21a) in said dryer fabric (12) at selected positions across the width of said dryer fabric (12) to produce longitudinally extending zones (18, 19, 20) in said dryer fabric (12) across the width thereof of different permeabilities, characterized in that said additional yarns are introduced in the dryer fabric (12) as stuffer picks (17, 17a, 21, 21a) laid in cross machine direction and being of a length shorter than the width of the dryer fabric (12).

13. The method claimed in claim 12 wherein said machine direction yarns, said cross machine direction yarns (14, 15) and said.stuffer picks (17, 17a, 21, 21a) are chosen from the class consisting of monofilament yarns, multifilament yarns, spun yarns and combinations thereof.

14. The method claimed in claim 12 wherein said stuffer picks (17, 17a, 21, 21a) are of a softness and stiffness up to that of said cross machine direction yarns (14, 15).

15. The method claimed in claim 12 including the steps of introducing a first group of said stuffer picks (17) into said dryer fabric (12) such that they extend from one longitudinal edge thereof toward the center thereof a predetermined distance and introducing into said dryer fabric (12) a second group of said stuffer picks (17) such that they extend from the other lateral edge thereof toward the center thereof a predetermined distance, the stuffer picks (17) of each of said groups being of the same length whereby to provide a dryer fabric (12) having two edge zones (18, 19) of lesser fluid permeability and a center zone (20) therebetween of greater fluid permeability.

16. The method claimed in claim 12 including the steps of introducing a first group of said stuffer picks (17, 17a) into said dryer fabric (12c) such that they extend from one longitudinal edge thereof toward the center thereof and introducing into said dryer fabric a second group of said stuffer picks (17, 17a) such that they extend from the other lateral edge thereof toward the center thereof, alternate ones of the stuffer picks (17a) of each of said first and second groups thereof being longer than the remaining stuffer picks (17) of said group, in each of said first and second groups said alternate longer stuffer picks (17a) being of the same length and said remaining stuffer picks (17) being of the same length, whereby to provide a dryer fabric (12c) having two edge zones (22, 23) of lesser fluid permeability, a center zone (24a) of higher fluid permeability and two intermediate zones (25a, 26a) of intermediate fluid permeability.

17. The method claimed in claim 15 including the step of introducing into said dryer fabric (12a) a third group of said stuffer picks (21) such that they extend between said stuffer picks (17) of said first and second groups.

18. The method claimed in claim 16 including the step of introducing into said dryer fabric (12b) a third group of said stuffer picks (21, 21a) such that they extend between said yarns (17, 17a) of said first and second groups.

19. The method claimed in claim 17 wherein said stuffer picks (21) of said third group have a diameter less than said stuffer picks (17) of said first and second groups.

20. The method claimed in claim 17 wherein said stuffer picks (21) of said third group are of less bulk than said stuffer picks (17) of said first and second groups.

21. The method claimed in claim 18 wherein said stuffer picks (21,21 a) of said third group have a diameter less than said stuffer picks (17, 17a) of said first and second groups.

22. The method claimed in claim 18 wherein said stuffer picks (21, 21a) of said third group are of less bulk than said stuffer picks (17, 17a) of said first and second groups.

## Patentansprüche

1. Trocknergewebe (12) zur Verwendung in einer Papiermaschine, welches aus in Maschinenrichtung verlaufenden Garnen (13) und aus quer zur Maschinenrichtung verlaufenden Garnen (14, 15) als mehrlagiges Gewebe gewebt ist, wobei in Maschinenrichtung verlaufenden Garne (13) längs der Breite des Trocknergewebes (12) gleichmäßige Abstände voneinander haben und wobei zusätzliche Garne (17, 17a, 21, 21a) in dem Trocknergewebe (12) an ausgewählten Positionen quer zur Breite des Trocknergewebes (12) angeordnet sind, um in Längsrichtung verlaufende Zonen (18, 19, 20) in dem Trocknergewebe (12) quer zur Breite desselben zur erzeugen, welche unterschiedliche Flüssigkeitsdurchlässigkeiten haben, dadurch gekennzeichnet, daß die zusätzlichen Garne Füllfäden (17, 17a, 21, 21a) sind, die quer zur Maschinenrichtung gelegt sind und eine Länge haben, die kürzer ist als die Breite des Trocknergewebes.

2. Die Struktur, die in Anspruch 1 beansprucht ist, bei der die in Maschinenrichtung verlaufenden Garne (13) und die quer zur Maschinenrichtung verlaufenden Garne (14, 15) und die Füllfäden (17, 17a, 21, 21a) aus der Klasse ausgewählt sind, die besteht aus: Monofilament-Garnen, Multifilament-Garnen, gesponnenen Garnen und Kombinationen derselben.

3. Die Struktur, die in Anspruch 1 beansprucht ist, bei der die Füllfäden (17, 17a, 21, 21a) eine Weichheit und Steifigkeit bis zu derjenigen der quer zur Maschinenrichtung verlaufenden Garne haben.

4. Die Struktur, die in Anspruch 1 beansprucht ist, welche eine erste und eine zweite Gruppe der Füllfäden (17) umfasst, wobei die Füllfäden (17) der ersten Gruppe in dem Trocknergewebe so angeordnet sind, daß sie sich über eine vorgegebene Strecke von der einen Längskante desselben in Richtung auf die Mitte desseiben erstrecken, wobei die Füllfäden (17) der zweiten Gruppe in dem Trocknergewebe (12) so angeordnet sind, daß sie sich über eine vorgegebene Strecke von der anderen Längskante desselben zur Mitte desselben erstrecken, wobei die Füllfäden (17) jeder dieser Gruppen dieselben Länge haben und wobei das Trocknergewebe (12) zwei Randzonen (18, 19) vom geringerer Flüssigkeitsdurchlässigkeit und eine dazwischenliegende Mittelzone von größerer Flüssigkeitsdurchlässigkeit aufweist.

5. Die Struktur, die in Anspruch 1 beansprucht ist, welche eine erste und eine zweite Gruppe von Füllfäden (17, 17a) aufweist, wobei die Füllfäden (17, 17a) der ersten Gruppe in dem Trocknergewebe (12c) so angeordnet sind, daß sie sich von einer Längskante desselben in Richtung auf die Mitte desselben erstrecken, wobei die Füllfäden (17, 17a) der zweiten Gruppe in dem Trocknergewebe so angeordnet sind, daß sie sich von der anderen Längskante desselben in Richtung auf die Mitte desselben erstrecken, wobei jeder zweite Füllfaden (17a) in der ersten und in der zweiten Gruppe länger ist als die restlichen Füllfäden (17) der betreffenden Gruppe, wobei in der ersten und zweiten Gruppe jeder zweite längere Füllfaden (17a) dieselbe Länge hat und wobei die verbleibenden Füllfäden (17) dieselbe Länge haben, wobei das Trocknergewebe (12a) zwei Randzonen (22, 23) geringerer Flüssigkeitsdurchlässigkeit, eine Mittelzone (24a) höherer Flüssigkeitsdurchlässigkeit und zwei Zwischenzonen (24a, 26a) mittlerer Flüssigkeitsdurchlässigkeit aufweist.

6. Die Strucktur, die in Anspruch 4 beansprucht ist, welche eine dritte Gruppe von Füllfäden (21) umfasst, wobei die Füllfäden (21) der dritten Gruppe in dem Trocknergewebe (12a) derart angeordnet sind, daß sie sich zwischen den Füllfäden (17) der ersten und der zweiten Gruppe erstrecken.

7. Die Struktur, die in Anspruch 5 beansprucht ist, welche eine dritte Gruppe von Füllfäden (21, 21a) umfasst, wobei die Füllfäden (21, 21a) dieser dritten Gruppe in dem Trocknergewebe (12b) so angeordnet sind, daß sie sich zwischen den Füllfäden (17, 17a) der ersten und der zweiten Gruppe von Garnen erstrecken.

8. Die Struktur, die in Anspruch 6 beansprucht ist, bei der die Füllfäden (21) der dritten Gruppe einen Durchmesser haben, der kleiner ist als der Durchmesser der Füllfäden (17) der ersten und der zweiten Gruppe.

9. Die Struktur, die in Anspruch 6 beansprucht ist, bei der die Füllfäden (21) der dritten Gruppe eine geringere Fülle haben als die Füllfäden (17) der ersten und der zweiten Gruppe.

10. Die Struktur, die in Anspruch 7 beansprucht ist, bei der die Füllfäden (21, 21a) der dritten Gruppe einen Durchmesser haben, der kleiner ist als der Durchmesser der Füllfäden (17, 17a) der ersten und der zweiten Gruppe.

11. Die Struktur, die in Anspruch 7 beansprucht ist, bei der die Füllfäden (21, 21a) der dritten Gruppe eine geringere Fülle haben als die Füllfäden (17, 17a) der ersten und der zweiten Gruppe.

12. Verfahren zur Herstellung eines Trocknergewebes (12) zur Verwendung in einer Papiermaschine, welches die (folgenden) Schritte umfasst: das Trocknergewebe (12) wird aus in Maschinenrichtung verlaufenden Garnen (13) und aus quer zur Maschinenrichtung verlaufenden Garnen (14,15) als mehrlagiges Gewebe gewebt, wobei die in Maschinenrichtung verlaufenden Garne (13) über die Breite des Trocknergewebes (12) in gleichmäßigen Abständen angeordnet werden, und in diseses Trocknergewebe (12) werden zusätzliche Grane (17, 17a, 21, 21a) an ausgewählten Positionen quer zur Breite des Trocknergewebes (12) eingeführt, um quer zum Breite des Trocknergewebes (12) in Längsrichtung verlaufende Zonen (18, 19, 20) mit unterschiedlichen Wasserdurchlässigkeiten zu erzeugen, dadurch gekennzeichnet, daß die zusätzlichen Garne in das Trocknergewebe (12) als Füllfäden (17, 17a, 21, 21a) eingeführt werden, welche quer zur Maschinenrichtung gelegt werden und eine Länge haben, die kürzer ist als die Breite des Trocknergewebes (12).

13. Das Verfahren, welches in Anspruch 12 beansprucht ist, bei dem die in Maschinenrichtung verlaufenden Garne, die quer zur Maschinenrichtung verlaufenden Garne (14, 15) und die Füllschäden (17, 17a, 21, 21a) aus der Klasse ausgewählt werden, die besteht aus: Monofilament-Garnen, Multifilament-Garnen, gesponnenen Garnen und Kombinationen derselben.

14. Das Verfahren, welches in Anspruch 12 beansprucht ist, bei dem die Füllfäden (17, 17a, 21, 21a) eine Weichheit und Steifigkeit bis zu derjenigen der quer zur Maschinenrichtung verlaufenden Garne (14, 15) haben.

15. Das Verfahren, welches in Anspruch 12 beansprucht ist, welches die (folgenden) Schritte umfasst: eine erste Gruppe von Füllfäden (17) wird so in das Trocknergewebe (12) eingeführt, daß die Füllfäden sich von einer Längskante desselben über eine vorgegebene Strecke in Richtung auf die Mitte desselben erstrecken, und in das Trocknergewebe (12) wird eine zweite Gruppe von Füllfäden (17) derart eingeführt, daß die Füllfäden sich von der anderen Längskante desselben über eine vorgegebene Strecke in Richtung auf die Mitte desselben erstrecken, wobei die Füllfäden (17) jeder der Gruppen dieselbe Länge haben, um dadurch ein Trocknergewebe (12) zu schaffen, welches zwei Randzonen (18, 19) geringerer Flüssigkeitsdurchlässigkeit und eine dazwischenliegende, mittlere Zone (20) größerer Flüssigkeitsdurchlässigkeit aufweist.

16. Das Verfahren, welches in Anspruch 12 beansprucht ist, welches die (folgenden) Schritte umfasst: die erste Gruppe von Füllfäden (17, 17a) wird derart in das Trocknergewebe (12c) eingeführt, daß sich die Füllfäden von einer Längskante desselben in Richtung auf die Mitte desselben erstrecken, und in das Trocknergewebe wird eine zweite Gruppe von Füllfäden (17, 17a) derart eingeführt, daß sich diese Füllfäden von der anderen Längskante desselben in Richtung auf die Mitte desselben erstrecken, wobei jeder zweite Füllfaden (17a) in der ersten und in der zweiten Gruppe länger ist als die restlichen Füllfäden (17) der betreffenden Gruppe, wobei in der ersten und in der zweiten Gruppe die zweiten, längeren Füllfäden (17a) dieselbe Länge haben und wobei die restlichen Füllfäden (17) dieselbe Länge haben, um auf diese Weise ein Trocknergewebe (12) herzustellen, welches zwei Randzonen (22, 23) geringerer Flüssigkeitsdurchlässigkeit, eine mittlere Zone (24a) höherer Flüssigkeitsdurchlässigkeit und zwei Zwischenzonen (25a, 26a) mittlerer Flüssigkeitsdurchlässigkeit aufweist.

17. Das Verfahren, welches in Anspruch 15 beansprucht ist, welches den Schritt umfasst, daß in das Trocknergewebe (12b) eine dritte Gruppe der Füllfäden (21,21a) derart eingeführt wird, daß diese Füllfäden (21, 21a) sich zwischen der Garnen (17, 17a) der ersten und der zweiten Gruppe (von Füllfäden) erstrecken.

18. Das Verfahren, welches in Anspruch 16 beansprucht ist, welches den Schritt umfasst, daß in das Trocknergewebe (12b) eine drite Gruppe der Füllfäden (21,21a) derart eingeführt wird, daß diese sich zwischen den Garnen (17, 17a) der ersten und der zweiten Gruppe erstrecken.

19. Das Verfahren, welches in Anspruch 17 beansprucht ist, bei dem die Füllfäden (21) der dritten Gruppe einen Durchmesser haben, der kleiner ist als der Durchmesser der Füllfäden (17) der ersten und der zweiten Gruppe.

20. Das Verfahren, welches in Anspruch 17 beansprucht ist, bei dem die Füllfäden (21) der dritten Gruppe eine geringere Fülle haben als die Füllfäden (17) der ersten und der zweiten Gruppe.

21. Das Verfahren, welches in Anspruch 18 beansprucht ist, bei dem die Füllfäden (21, 21a) der dritten Gruppe einen Durchmesser haben, der kleiner ist als der Durchmesser der Füllfäden (17, 17a) der ersten und der zweite Gruppe.

22. Das Verfahren, welches in Anspruch 18 beansprucht ist, bei dem die Füllfäden (21, 21a) der dritten Gruppe eine geringere Fülle haben als die Füllfäden (17, 17a) der ersten und der zweiten Gruppe.

## Revendications

1. Tissu sécheur tissé (12) pour machine à papier, formé de filés sens-machine (13) et de filés sens-travers-machine (14,15) suivant une armure à plusieurs couches, les filés sens-machine (13) étant espacés de manière uniforme suivant la largeur du tissu sécheur (12), et des filés supplémentaires (17, 17a, 21, 21a) étant prévus dans le tissu sécheur (12) en des positions choisies suivant la largeur du tissu sécheur (12) pour créer des zones longitudinales (18,19,20) dans ce tissu sécheur (12), ayant, suivant la largeur de celui-ci, des perméabilités différentes aux fluides, caractérisé en ce que les filés supplémentaires sont des trames ou duites de fourrure (17, 17a, 21, 21a) disposées dans le sens-travers-machine et étant d'une longueur inférieure à la largeur du tissu sécheur (12).

2. Structure suivant la revendication 1, caractérisée en ce que les filés sens-machine (13, les filés sens-travers-machine (14, 15) et les trames de fourrure (17, 17a, 21, 21a) sont choisis dans la classe comprenant des fils monobrins, des fils multibrins, des filés et leurs combinaisons.

3. Structure suivant la revendication 1, caractérisée en ce que les trames de fourrure (17, 17a, 21,21a) sont d'une douceur et d'une raideur allant jusqu'à celles des fils sens-travers-machine.

4. Structure suivant la revendication 1, caractérisée en ce qu'elle comprend un premier et un second groupe de trames de fourrure (17), les trames de fourrure (17) du premier groupe étant localisées de telle sorte, dans le tissu sécheur (12), qu'elles s'étendent depuis un bord longitudinal de ce tissu sur une distance prédéterminée en direction de son centre, le second groupe de trames de fourrure (17) étant localisé de telle manière, dans le tissue sécheur (12), que ces trames s'étendent depuis l'autre bord longitudinal du tissu en direction de son centre sur und distance prédéterminée, les trames de fourrure (17) de chacun de ces groupes étant de la même longueur, le tissu sécheur (12) comportant deux zones marginales (18, 19) d'une perméabilité moindre aux fluides et une zone central (20) prévue entre les deux zones précédentes et d'une perméabilité plus élevée aux fluides.

5. Structure suivant la revendication 1, caractérisée en ce qu'elle comprend un premier et un second groupe de trames de fourrure (17, 17a), les trames de fourrure (17, 17a), du premier groupe étant localisées de telle manière, dans le tissu sécheur (12c), qu'elles s'étendent depuis un bord longitudinal de ce tissu en direction du centre de celui-ci, les trames de fourrure (17, 17a) du second groupe étant localisées de telle manière, dans le tissu séchir (12c), qu'elles s'étendent depuis l'autre bord longitudinal de ce tissue en direction de son centre, les trames alternées parmi les trames de fourrure (17a) de chacun du premier et du second groupe étant plus longues que les trames de fourrure restantes (17) de ce groupe, les trames de fourrure (17a) plus longues alternées, dans chacun des premier et second groupes susdits, étant de la même longueur, tandis que les trames de fourrure restantes (17) sont également de la même longuer le tissu sécheur (12a) comportant deux zones marginales (22, 23) d'une perméabilité moindre aux fluides, une zone centrale (24a) d'une perméabilité plus élevée aux fluides, et deux zones intermédiaires (24a, 26a) d'un perméabilité intermédiaire aux fluides.

6. Structure suivant la revendication 4, caractérisée en ce qu'elle comprend un troisième groupe de trames de fourrure (21), ces trames de fourrure (21) du troisième groupe étant localisées de telle manière, dans le tissu sécheur (12a), qu'elles s'étendent entre les trames de fourrure susdites (17) du premier groupe et du second groupe.

7. Structure suivant la revendication 5, caractérisée en ce qu'elle comprend un troisième groupe de trames de fourrure (21, 21a), ces trames de fourrure (21, 21a) du troisième groupe étant localisée de telle manière, dans le tissu sécheur (12b), qu'elles s'étendent entre les trames de fourrure (17, 17a) du premier et du second groupe de filés.

8. Structure suivant la revendication 6, caractérisée en ce que les trames de fourrure (21) du troisième groupe ont un diamètre inférieur à celui des trames de fourrure (17) du premier et du second groupe.

9. Structure suivant la revendication 6, caractérisée en ce que les trames de fourrure (21) du troisième groupe sont d'un volume moindre que les trames de fourrure (17) du premier et du second groupe.

10. Structure suivant la revendication 7, caractérisée en ce que les trames de fourrure (21, 21a) du troisième groupe ont un diamètre inférieur à celui des trames de fourrure (17, 17a) du premier et du second groupe.

11. Structure suivant la revendication 7, caractérisée en ce que les trames de fourrure (21, 21a) du troisième groupe sont d'un volume moindre que les trames de fourrure (17, 17a) du premier et du second groupe.

12. Procédé de fabrication d'un tissu sécheur (12) à utiliser dans une machine à papier, comprenant les phases de tissage de ce tissu sécheur (12) en fils sens-machine (13) et en fils sens-travers-machine (14,15) suivant une armure à plusieurs couches, les fils sens-machine (13) étant espacés de manière uniforme suivant la largeur du tissu sécheur (12), et d'introduction de fils supplémentaires (17, 17a, 21, 21a) dans ce tissu sécheur (12) en des positions choisies suivant la largeur de ce tissu sécheur (12) pour créer des zones longitudinales (18, 19, 20) dans ce tissu sécheur (12), suivant sa largeur, qui ont des perméabilités différentes, caractérisé en ce que les fils supplémentaires susdits sont introduits dans le tissu sécheur (12) sous forme de trames ou duites de fourrure (17, 17a, 21, 21a) disposées dans le sens-travers-machine et qui sont d'une longueur inférieure à la largeur du tissu sécheur (12).

13. Procédé suivant la revendication 12, caractérisé en ce que les fils sens-machine, les fils sens-travers-machine (14, 15) et les trames de fourrure (17, 17a, 21, 21a) sont choisies dans la classe comportant des fils monobrins, des fils multibrins, des filés, et leurs combinaisons.

14. Procédé suivant la revendication 12, caractérisé en ce que les trames de fourrure (17, 17a, 21, 21a) sont d'une douceur et d'une raideur allant jusqu'à celles des fils sens-travers-machine (14, 15).

15. Procédé suivant la revendication 12, caractérisé en ce qu'il comprend les phases d'introduction d'un premier groupe de trames de fourrure (17) dans le tissu sécheur (12) de manière qu'elles s'étendent depuis un bord longitudinal de ce tissu sur une distance prédéterminée en direction de son centre, et d'introduction, dans ce tissu sécheur (12), d'un second groupe de trames de fourrure (17), de manière qu'elles s'étendent depuis l'autre bord latéral du tissu sur une distance prédéterminée en direction de son centre, les trames de fourrure (17) de chacun de ces groupes étant de la même longueur de manière à former un tissu sécheur (12) comportant deux zones marginales (18, 19) d'une perméabilité moindre aux fluides et une zone centrale (20) comprise entre les zones précédentes et d'une plus grande perméabilité aux fluides.

16. Procédé suivant la revendication 12, caractérisé en ce qu'il comprend les phases d'introduction d'un premier groupe de trames de fourrure (17, 17a) dans le tissu sécheur (12c) de manière qu'elles s'étendent depuis un bord longitudinal de ce tissu sur une distance prédéterminée en direction de son centre, et d'introduction, dans ce tissu sécheur, d'un second groupe de trames de fourrure (17, 17a) de manière qu'elles s'étendent depuis l'autre bord latéral de ce tissu en direction de son centre, des trames alternées parmi les trames de fourrure (17a) de chacun du premier et du second groupe étant plus longues que les trames de fourrure restantes (17) de ce groupe, les trames de fourrure (17a) plus longues et alternées, dans chacun de ce premier et de ce second groupe, étant de la même longueur, tandis que les trames de fourrure restantes (17) sont également de la même longueur, de manière à former un tissu sécheur (12c) comportant deux zones marginales (22, 23) d'une perméabilité moindre aux fluides, une zone centrale (24a) d'un perméabilité plus élevée aux fluides, et deux zones intermédiaires (25a, 26a) d'une perméabilité intermédiaire aux fluides.

17. Procédé suivant la revendication 15, caractérisé en ce qu'il comprend la phase d'introduction, dans le tissu sécheur (12a) susdit, d'un troisième groupe de trames de fourrure (21) de manière que celles-ci s'étendent entre les trames de fourrure (17) du premier et du second groupe.

18. Procédé suivant la revendication 16, caractérisé en ce qu'il comprend la phase d'introduction, dans le tissu sécheur (12b) susdit, d'un troisième groupe de trames de fourrure (21, 21a) de manière que celles-ci s'étendent entre les fils (17, 17a) du premier et du second groupe.

19. Procédé suivant la revendication 17, caractérisé en ce que les trames de fourrure (21) du troisième groupe ont un diamètre inférieur à celui des trames de fourrure (17) du premier et du second groupe.

20. Procédé suivant la revendication 17, caractérisé en ce que les trames de fourrure (21) du troisième groupe sont d'un volume moindre que les trames de fourrure (17) du premier et du second groupe.

21. Procédé suivant la revendication 18, caractérisé en ce que les trames de fourrures (21, 21a) du troisième groupe ont un diamètre inférieur à celui des trames de fourrure (17, 17a) du premier et du second groupe.

22. Procédé suivant la revendication 18, caractérisé en ce que les trames de fourrure (21, 21a) du troisième groupe sont d'un volume moindre que les trames de fourrure (17, 17a) du premier et du second groupe.
